

Nov. 2, 1926.

1,605,197

W. H. ANFIELD

COMPOSITION FLOOR AND METHOD OF MAKING THE SAME

Filed June 23, 1924



INVENTOR:  
WILLIAM HENRY ANFIELD  
BY Edward G. Longan  
ATTORNEY

## UNITED STATES PATENT OFFICE.

WILLIAM HENRY ANFIELD, OF ST. LOUIS, MISSOURI.

## COMPOSITION FLOOR AND METHOD OF MAKING THE SAME.

Application filed June 23, 1924. Serial No. 721,930.

My invention relates to improvements in composition floors and method of making the same, and has for its primary object the construction of a concrete floor whereby cracking is practically eliminated, and the construction of such a floor is of less expense than similar floors now in use.

In the drawings:

Fig. 1 is a fragmental perspective view of a portion of my floor and base board when completed;

Fig. 2 is a fragmental section of the same in position when in use.

In the construction of my floor I commence with the concrete floor which is put in by the builder and is indicated by 3 which is the base or foundation for my floor. This base 3 is constructed of concrete and properly reinforced in the usual way. Beginning with the concrete flooring as put in by the builder, I then lay over this concrete base a layer of sand and cement and finely crushed stone 4. This is for the purpose of leveling up the foundation 3, as it is well known that the cement floor put in by the builder is generally left in a rough and crude state. After I have placed the layer 4 of sand, cement and finely crushed stone on the concrete base 3 I then apply my improved flooring in the following manner:—

I take a mass of concrete formed of sand, cement and chipped rock, such as marble or granite, and apply it on the layer 4 and completely cover the space to be floored, and make the same of the required thickness, the floor being indicated by 5. The floor or layer 5 is properly smoothed down and leveled off and permitted to harden and to form a monolithic floor, that is, it is put on and permitted to harden as one continuous solid sheet. After this layer or floor 5 has hardened it is then surfaced. After it has been surfaced I take a suitable tool or instrument and form channels 6 through the layer or floor 5 and partly into the layer 4. These channels may be of any suitable or desired width, shape or number so as to give the floor the desired blocked-off appearance. After these channels have been formed I apply oil by means of a brush in the channels, slightly coating the channel walls with oil, and after this operation I fill in the channels with "grout", that is, a thin mixture of cement and water. I then permit the grout to hard-

en and resurface the floor again. The grout 65 may be mixed with any colored pigment desired.

By forming the channels 6 or cutting up the floor as it were into slabs after it has been laid and finished and filling in the channels with grout, cracking of the floor by settling is prevented, and cracking by expansion is eliminated.

I can also form by my improved method a neater appearance because the channels can 65 be cut smooth and straight and the joints, after the channels are filled in, are true and accurate. I have found in practice that the making of a concrete floor out of concrete slabs is expensive because the slabs must be 70 made at the factory and taken to the place to be used and laid and great difficulty has been experienced in truing up the joints.

Great disadvantage has also been experienced in making this kind of a floor and 75 leaving it in one solid piece, in which cases, expansion and settling in a great number of cases has ruined the floor and it has to be torn up. My improved floor can be completely made and laid on the job thus obviating the necessity of making the slabs at 80 one place and hauling them to the job and laying them.

In the construction of my improved floor I form at the same time with the floor proper 85 a base 7, this is formed integral with the floor proper and can be made any height or shape desired, and when the floor is scored the base is also scored and grouted in, as 90 illustrated in Fig. 1.

In practice I form the levelling layer 4 of sand and cement, properly mixed, or sand, cement and crushed stone, properly mixed. When I use sand and cement I use them in the following proportions, about three sacks 95 of sand to one of cement; and when I use the three I use about one sack of cement, one sack of crushed stone and two sacks of sand, properly mixed with water.

In practice in forming the floor layer 5 100 I use marble chips and cement, properly mixed, in about the following proportions, three sacks of marble chips to one of cement, properly mixed with water, which is worked down until the top surface shows about 85% 105 marble.

My improvement especially relates to what is commercially known as terrazzo floor.

Having fully described my invention, what I claim is:—

1. The improvement in the art of concrete flooring which consists in forming a base layer, applying to said base a plastic mass of sand and cement, applying on said mass of sand and cement after it has set a monolithic layer, forming channels through the monolithic layer and said plastic mass after the same has hardened, and filling said channels with a plastic self-hardening filler. 5
2. The improvement in the art of floor construction which consists in forming a concrete base, applying on said concrete base a plastic mass of sand and cement, applying to said mass after it has set a coating of the desired thickness composed of cement, water and chipped stone and permitting the same to harden as one monolithic layer, surfacing 10 said monolithic layer, forming channels through said monolithic layer and into the mass beneath it, coating said channels with oil, filling said channels with a relatively thin solution of cement and water and permitting the same to harden, and lastly refinishing the same. 15
3. The herein described method of producing a concrete floor, consisting in laying a terrazzo concrete surface of the proper thickness, cutting kerfs or grooves in the terrazzo surface after it is hardened, and filling in the said kerfs or grooves with grout. 20
4. The herein described method of making concrete floor, consisting in laying a monolithic layer of terrazzo of the desired thickness and permitting the same to harden, and then finishing the surface thereof, cutting kerfs or grooves in the said layer and filling 25 said kerfs or grooves with grout material. 25
5. The herein described method of pro- 30
- ducing a floor, consisting in applying to a concrete base a monolithic layer of terrazzo concrete and permitting it to harden, subdividing the said hardened monolithic layer of terrazzo concrete by cutting grooves there- 45 in and then filling said grooves with material. 50
6. The improvement in the art of floor construction which consists in forming a concrete base, applying on said concrete base a plastic mass of sand and cement, applying to said mass after it has set a coating of the desired thickness composed of cement, water and chipped stone and permitting the same to harden as one monolithic layer sur- 55
- 60
- 65
- 70
- 75
- 80
- 85
- 90
- 95

In testimony whereof, I have signed my name to this specification.

WILLIAM HENRY ANFIELD.